

Patented May 27, 1947

2,421,001

# UNITED STATES PATENT OFFICE

2,421,001

## COATING COMPOSITION COMPRISING CELLULOSE-ACETO-PROPIONATE AND AN ALKYD RESIN

Harry K. Ash, Cincinnati, Ohio, assignor to Interchemical Corporation, New York, N. Y., a corporation of Ohio

No Drawing. Application July 1, 1943.  
Serial No. 493,113

1 Claim. (Cl. 260—16)

1

This invention aims to provide a temporary protective coating for metal and similar impervious surfaces, characterized by the properties of unusual strength and resistance to abrasion, coupled with the ability to strip cleanly from a metal surface even after a prolonged period of time.

In the metal working field, there has existed a considerable demand for a temporary protective coating which would serve to protect the metal against abrasion until the metal object is actually put into use, but which is easily removable from the metal surface thereafter. This demand has existed with respect to decorative metal objects, where it is desired to retain the metallic luster and sheen of a polished surface during packing, shipping and handling prior to actual installation, or sale to a customer for use in the home. A more important use has been in the commercial field, where it is desired to protect a portion of a metal surface from damage during machining or working of the rest of the surface, or to protect an entire surface from surface marring while a piece of metal is bent, or otherwise deformed.

It has been proposed to use a wide variety of compositions for the production of temporarily adherent films. Transparent foils made from Cellophane, cellulose derivatives and resins have been suggested, but the task of fitting preformed foils onto irregularly shaped objects has made this approach unsuccessful. Various coating compositions which deposit a film have likewise been tried, including rubber latex, and cellulose ester and ether lacquers. Many of the compositions require a multiple treatment of the surface to obtain the desired result; this is highly undesirable from the cost standpoint. Other compositions are too soft to withstand abrasion; others do not strip cleanly from the metallic surface, either because of adhesion, or because the films tear on attempted removal; and many others which strip for a few days lose the power to strip on aging.

I have discovered a new type of coating composition which in one application produces on metal a temporarily protective film which is characterized by high resistance to abrasion, and the ability to strip cleanly from the metal even after prolonged standing. My compositions consist essentially of solutions of cellulose aceto-propionate, in solvent combinations consisting of at least 75% active solvent for the cellulose ester, the compositions being further characterized by a minimum viscosity of 50 seconds in a No. 4 Ford cup at 70° F.

According to my investigations, cellulose aceto-propionate is unique among the cellulose derivatives in that it yields films with the optimum combination of film strength and strippability

2

from metal. Other cellulose derivatives either tend to adhere more to metal, or to yield films of lower strength.

The cellulose aceto-propionate which I use may be of any of the commercial grades available. These generally contain about 15.5% acetyl and 31.5% propionyl content, and vary in viscosity from low to high. The low viscosity ester has a viscosity of 2 seconds, measured by the time required for a  $\frac{1}{8}$  inch diameter steel ball to fall in a 1 inch tube through a 10 inch depth of a 2% solution in acetone at 25° C.; the high viscosity material has a 30 second viscosity. I prefer the low viscosity material, as it gives more concentrated solutions and thicker films; but the high viscosity product can be used.

Preferably, the aceto-propionate should be plasticized. Unplasticized films will strip satisfactorily, but lack the versatility of plasticized films. However, in order to keep the film sufficiently hard to withstand abrasion, the plasticizer should preferably not exceed the weight of the cellulose ester.

Some resin may be used in the composition, so long as not so much resin is used that the film adheres too strongly to the surface coated. The amount which may be used varies depending upon the resin used and the adhesion imparted to the film thereby. In general, the amount of resin and plasticizer present should not substantially exceed the amount of cellulose aceto-propionate. I prefer to use plasticizing resins such as alkyd resins, plasticizing chlorinated diphenyls, plasticizing vinyl resins, and the like.

A stripping agent may be used if desired. While not necessary for many metal surfaces, the use of such an agent is desirable, particularly with easily wetted metal such as unpolished steel. Typical stripping agents are the citrate of the mono-ethyl ether of diethylene glycol (Carbitol citrate) and "Alumileaf" (a proprietary product sold for improving the leafing of aluminum paint). When used, they are ordinarily present in amounts varying from a few (about three) tenths of a percent to a few (about three) percent of the composition.

A most important consideration in my new compositions stems from my discovery of the fact that a stripping lacquer, in order to be satisfactory, must deposit a film of at least about 1 mil in dry thickness; thinner films do not strip properly, no matter how strong the film is. This necessity for a thick film in one coat requires high solids in the lacquer. High solids are ordinarily attained by the use of a low viscosity cellulose derivative combined with large quantities of plasticizer or resin. Such normal high solids lacquers are, however, not useable as stripping lacquers because of their formulation, being generally too adherent, as well as either soft (too much

## 3

plasticizer) or brittle (too much resin) for proper stripping.

Hence, I produce high solids by the use of solvents, of which at least 75% are active solvents for the cellulose aceto-propionate. These solvents not only produce a thinner solution at a given solids content, but they have two other effects—they insure maximum film strength by eliminating any blushing tendency, and they permit spraying at relatively high viscosity, thus permitting the use of higher solids again. I have found that my compositions, in order to produce films of at least about 1 mil in thickness, should have a minimum viscosity of 50 seconds in a No. 4 Ford cup at 70° F. Spraying lacquers may go up to about 100 seconds in viscosity; above that, very poor spraying results. Brushing lacquers may be as high as 200 seconds in viscosity. These viscosities compare with the approximately 20 second viscosities preferred in ordinary spraying lacquers.

Typical examples of my invention are the following:

## Example 1

|                                                                                                           | Parts by weight |
|-----------------------------------------------------------------------------------------------------------|-----------------|
| Hercose AP low viscosity (cellulose aceto propionate low viscosity—15.5% acetyl, 31.5% propionyl content) | 7.35            |
| Alkyd resin                                                                                               | 7.35            |
| Ethyl acetate                                                                                             | 35.30           |
| Butyl acetate                                                                                             | 45.00           |
| Cellosolve acetate hydroxyethyl acetate                                                                   | 5.00            |

The alkyd resin is prepared by reacting—

|                    | Parts by weight |
|--------------------|-----------------|
| Sebacic acid       | 37.5            |
| Succinic anhydride | 28.6            |
| Ethylene glycol    | 19.3            |
| Glycerol           | 14.6            |

to an acid number of about 70.0. It is essentially a plasticizing resin.

The lacquer has a viscosity of 60 seconds in a No. 4 Ford cup at 70° F.; the solids are relatively high for the viscosity and high ratio of cellulose ester, largely because the solvent is all active solvent for the ester. Films obtained by spraying on metal are permanently strippable.

## Example 2

|                                                        | Parts by weight |
|--------------------------------------------------------|-----------------|
| Tricresyl phosphate                                    | 5.65            |
| #1254 Aroclor (chlorinated diphenyl 54% chlorine)      | 2.80            |
| Carbitol citrate                                       | 2.00            |
| Ethyl acetate                                          | 40.00           |
| Butyl acetate                                          | 34.45           |
| Hercose AP low viscosity                               | 8.90            |
| Vinylite A. Y. A. F. (low viscosity polyvinyl acetate) | .90             |
| Cellosolve acetate                                     | 5.30            |

This product differs from that of Example 1 in containing carbitol citrate, a stripping agent.

## Example 3

The product of Example 2 may be colored by the use of dye solutions (e. g. alcohol soluble dyes in alcohol) or by the use of a very small amount of pigment (e. g. 0.1% of phthalocyanine blue or green).

## Example 4

|                     | Parts by weight |
|---------------------|-----------------|
| Paste:              |                 |
| Zinc chromate       | 57.49           |
| Tricresyl phosphate | 42.06           |

Grind two runs on a three-roll mill.

## 4

|                                                             | Parts by weight |
|-------------------------------------------------------------|-----------------|
| Paste                                                       | 5.40            |
| #1248 Aroclor (chlorinated diphenyl—48% chlorine)           | 6.00            |
| 5 Ethyl acetate                                             | 38.23           |
| Butyl acetate                                               | 33.93           |
| Cellosolve acetate                                          | 5.07            |
| Hercose AP low viscosity (cellulose aceto-propionate)       | 8.51            |
| 10 Vinylite A. Y. A. F.                                     | .86             |
| Alumileaf                                                   | 2.00            |
| Blue dye solution (Geigy acid pure blue R Supra in alcohol) | Trace           |

This material has rust-inhibitive properties.

|                                                       | Parts by weight |
|-------------------------------------------------------|-----------------|
| Hercose AP low viscosity (cellulose aceto-propionate) | 9.71            |
| 20 Dibutyl phthalate                                  | .60             |
| #1248 Aroclor                                         | 1.83            |
| Alumileaf                                             | 2.00            |
| Cellosolve acetate                                    | 5.02            |
| Ethyl acetate                                         | 44.77           |
| 25 Butyl acetate                                      | 36.07           |

This product is low in plasticizer and high in cellulose derivative—it has unusually high tensile strength.

The small amount of pigment shown in Example 3 has little effect on the film; however, the 3% of pigment in Example 4 improves the ability of the film to withstand drawing and forming. Where it is desired to get such an improvement in properties, I may add a small amount (1 to 5%) of inert extender pigment, with or without a smaller amount of color pigment. This produces a film which can be marked with a pencil, etc. for lay-out purposes. A typical example is the following:

## Example 5

|                                                                                                              | Parts by weight |
|--------------------------------------------------------------------------------------------------------------|-----------------|
| Santocel (silica aerogel)                                                                                    | 10.01           |
| Surfex (calcium carbonate)                                                                                   | 2.88            |
| 45 Hercose AP low viscosity (cellulose aceto-propionate low viscosity—15.5% acetyl, 31.5% propionyl content) | 4.47            |
| Alkyd resin of Example 1                                                                                     | 4.47            |
| 50 Ethyl acetate                                                                                             | 32.34           |
| Butyl acetate                                                                                                | 41.20           |
| Cellosolve acetate                                                                                           | 4.63            |

100.00

55 are ground in a mill to a smooth paste.

|                                                                                                           | Parts by weight |
|-----------------------------------------------------------------------------------------------------------|-----------------|
| Above paste                                                                                               | 15.00           |
| Hercose AP low viscosity (cellulose aceto-propionate low viscosity—15.5% acetyl, 31.5% propionyl content) | 6.25            |
| 60 Alkyd resin of Example 1                                                                               | 6.25            |
| Ethyl acetate                                                                                             | 29.75           |
| Butyl acetate                                                                                             | 38.25           |
| Cellosolve acetate                                                                                        | 4.25            |
| 65 Chrome green pigment paste                                                                             | .25             |

100.00

70 Other extenders which can be used include various clays, magnesium silicate, barytes in various forms, calcium sulphate in various forms, diatomaceous earths, and similar inerts.

The examples can be multiplied indefinitely without departing from the scope of the invention, which is defined in the claim.

## I claim:

A stripping lacquer which will deposit a permanently strippable film at least 1 mil thick in a single spray application and which is characterized by a viscosity of about 60 seconds in a No. 4 Ford cup at 70° F., which consists essentially of a binder comprising the following ingredients in parts by weight:

Cellulose aceto-propionate of approximately 15.5% acetyl and 31.5% propionyl content ----- 7.35

Alkyd resin ----- 7.35

and a solvent for such binder comprising the following ingredients in parts by weight: 15

Butyl acetate ----- 45.00

Ethyl acetate ----- 35.30

Hydroxyethyl acetate ----- 5.00

said alkyd resin being prepared by reacting the following ingredients in parts by weight:

5 Sebacic acid ----- 37.5  
Succinic anhydride ----- 28.6  
Ethylene glycol ----- 19.3  
Glycerol ----- 14.6

HARRY K. ASH.

## REFERENCES CITED

The following references are of record in the file of this patent:

## 10 UNITED STATES PATENTS

| Number    | Name     | Date          |
|-----------|----------|---------------|
| 2,186,454 | Gloor    | Jan. 9, 1940  |
| 2,170,416 | Klinger  | Aug. 22, 1939 |
| 1,934,824 | Schwalbe | Nov. 14, 1933 |

## FOREIGN PATENTS

| Number  | Country | Date           |
|---------|---------|----------------|
| 736,429 | France  | Sept. 19, 1932 |

## 20 OTHER REFERENCES

Gloor, pages 690-696, Ind. and Eng. Chem., June 1937.

## Certificate of Correction

Patent No. 2,421,001.

May 27, 1947.

HARRY K. ASH

It is hereby certified that errors appear in the printed specification of the above numbered patent requiring correction as follows: Column 3, line 62, for "carbitol" read *Carbitol*; line 72, Example 4, for "57.49" read 57.94; and that the said Letters Patent should be read with these corrections therein that the same may conform to the record of the case in the Patent Office.

Signed and sealed this 5th day of August, A. D. 1947.

[~~SEAL~~]

LESLIE FRAZER,  
First Assistant Commissioner of Patents.

## I claim:

A stripping lacquer which will deposit a permanently strippable film at least 1 mil thick in a single spray application and which is characterized by a viscosity of about 60 seconds in a No. 4 Ford cup at 70° F., which consists essentially of a binder comprising the following ingredients in parts by weight:

Cellulose aceto-propionate of approximately 15.5% acetyl and 31.5% propionyl content ----- 7.35

Alkyd resin ----- 7.35

and a solvent for such binder comprising the following ingredients in parts by weight: 15

Butyl acetate ----- 45.00

Ethyl acetate ----- 35.30

Hydroxyethyl acetate ----- 5.00

said alkyd resin being prepared by reacting the following ingredients in parts by weight:

5 Sebacic acid ----- 37.5  
Succinic anhydride ----- 28.6  
Ethylene glycol ----- 19.3  
Glycerol ----- 14.6

HARRY K. ASH.

## REFERENCES CITED

The following references are of record in the file of this patent:

## 10 UNITED STATES PATENTS

| Number    | Name     | Date          |
|-----------|----------|---------------|
| 2,186,454 | Gloor    | Jan. 9, 1940  |
| 2,170,416 | Klinger  | Aug. 22, 1939 |
| 1,934,824 | Schwalbe | Nov. 14, 1933 |

## FOREIGN PATENTS

| Number  | Country | Date           |
|---------|---------|----------------|
| 736,429 | France  | Sept. 19, 1932 |

## 20 OTHER REFERENCES

Gloor, pages 690-696, Ind. and Eng. Chem., June 1937.

## Certificate of Correction

Patent No. 2,421,001.

May 27, 1947.

HARRY K. ASH

It is hereby certified that errors appear in the printed specification of the above numbered patent requiring correction as follows: Column 3, line 62, for "carbitol" read *Carbitol*; line 72, Example 4, for "57.49" read 57.94; and that the said Letters Patent should be read with these corrections therein that the same may conform to the record of the case in the Patent Office.

Signed and sealed this 5th day of August, A. D. 1947.

[~~SEAL~~]

LESLIE FRAZER,  
First Assistant Commissioner of Patents.